

## UNITED STATES PATENT OFFICE.

RENÉ CLAVEL, OF BASEL, SWITZERLAND.

## PROCESS OF DYEING CELLULOSE ACETATES.

No Drawing.

Application filed October 5, 1922. Serial No. 592,604.

*To all whom it may concern:*

Be it known that I, RENÉ CLAVEL, a citizen of the Swiss Republic, of Basel, Switzerland, have invented a certain new and useful Improved Process of Dyeing Cellulose Acetates, of which the following is a specification.

This invention relates to the dyeing of cellulose acetates in artificial silk, film or other form, in black shades.

In the specification of my United States Patent No. 1,448,432, it is stated and shown that certain groups in dyestuffs are capable of imparting to the dyestuffs containing them an increased affinity for the acetyl celluloses in artificial silk or other form, as such dyestuffs go into chemical reaction or present some other favourable physical condition relatively to the acetyl celluloses, it being immaterial whether these dyestuffs are in dissolved or undissolved form in the dye-baths. Amongst these active groups there were mentioned: amido, imino, imide-, and acidylamino groups (H-N-CO.R, in which R stands for alkyl or aryl). Amongst others, aniline black was given as an example of a dyestuff with active groups. Owing to its active groups this dyestuff can be brought into the fibre direct or in suspended form, but better by impregnating the fibre with aniline hydrochloride and developing. Technical working in the latter case has shown, however, that in spite of the cheapness of this aniline black, the fibre is sometimes affected in sympathy, so that it was of advantage to find a development black which would fulfil the textile demands in every respect. As a possible development black, diphenylamine containing two active groups was investigated, and it was found that with this the method of application usual with cotton was not suitable for acetyl celluloses, such for example as artificial silks, as only dull, uneven black dyeing of the goods was obtained.

In further constructive development, a process has now been found which is believed to fulfil all the technical requirements, as acetate silk fibres for example are neither weakened nor suffer in lustre by it, and moreover it enables any dye works which are not equipped for aniline black dyeing, to obtain nevertheless a handsome deep black similar to aniline black.

According to the invention cellulose acetates are dyed with diphenyl black base in

presence of an aliphatic carboxylic acid or acids, with or without soluble chloride salts, and with or without protective colloids, and developed.

The following examples illustrate how the invention may be carried out, but it will be understood that these are given by way of example only, and can be varied greatly without departing from the spirit of the invention.

*Example A.*

To dye 1 kg. of acetate silk, stock solutions are first prepared as follows:

Stock solution I: 200 gr. diphenyl black base, 250 cc. lactic acid 50%, 550 cc. acetic acid 50%, and the whole diluted to 1250 cc. with water.

The diphenyl black base is dissolved in the acids by warming and diluted as stated.

Stock solution II: 125 gr. aluminium chloride, 30° Bé., 125 gr. chromium chloride, 30° Bé., 20 gr. cupric chloride 40° Bé., 150 gr. sodium chloride in 60 cc. water, and the whole is made up to 1250 cc. solution.

Dyebath: This is prepared so that the weight of the diphenyl black base corresponds to 12 per cent of the weight of the goods.

Example: Dyebath for 1 kg. acetyl cellulose—750 cc. stock solution I, 750 cc. stock solution II, the whole diluted with water to about 4½-6½ litres.

Method of operation: The dyeing is performed in the cold. The goods are turned two to three times in the bath and soaked for half an hour. They are then removed from the bath and whizzed.

Developing: The oxidation or development is effected by placing the goods in a drying room at 80° C., preferably turning the goods on the rods once or twice during about an hour. After the development time mentioned the goods are washed twice, soaped at 50-60° C., then rinsed with two soft waters and one hard water and soured.

*Example B.*

One may also work as follows:

Stock solution: 200 gr. diphenyl black base, 500 cc. 80% acetic acid, 500 cc. water.

To dye 1 kg. cellulose acetate silk black, one half of this stock solution is taken, diluted with 20 liters of water and 2 liters of boiled off liquor (the well known liquor resulting from the "boiling-off" or degum-

ming of raw natural silk with soap solutions) are added. This dye bath is warmed to 50° C. and the goods are turned in the bath for about an hour. Then 50 grams of sodium acetate are added to the bath and the goods are treated in it for about an hour more at 60° C. They are then given a short rinsing and oxidized or developed in a second bath.

Developing bath: This consists of 20 liters

10 water, 100 gr. ammonium persulphate.

The goods are oxidized for about an hour. They are then washed, soaped at 50° C., rinsed with soft water and with hard water, and brightened.

15 One can however also work by developing in the exhausted dyebath, with careful addition of oxidizing agents such as hypochlorite, chloride of lime, persulphate or perborate.

20 What I claim and desire to secure by Letters Patent is:—

1. Process for dyeing acetyl cellulose in black shades, comprising treating the acetyl cellulose with diphenyl black base in presence of at least one aliphatic carboxylic acid 25 and developing the dye on the acetyl cellulose.

2. Process for dyeing acetyl cellulose in black shades, comprising treating the acetyl cellulose with diphenyl black base in presence of at least one aliphatic carboxylic acid and at least one soluble chloride salt, and developing the dye on the acetyl cellulose.

3. Process for dyeing acetyl cellulose in 30 black shades, comprising treating the acetyl cellulose with diphenyl black base in presence

ence of at least one aliphatic carboxylic acid and protective colloid, and developing the dye on the acetyl cellulose.

4. Process for dyeing acetyl cellulose in 40 black shades, comprising treating the acetyl cellulose with diphenyl black base in presence of at least one aliphatic carboxylic acid, at least one soluble chloride salt, and protective colloid, and developing the dye on the 45 acetyl cellulose.

5. Process for dyeing acetyl cellulose in black shades, comprising treating the acetyl cellulose with diphenyl black base in presence of acetic acid and developing the dye 50 on the acetyl cellulose.

6. Process for dyeing acetyl cellulose in black shades, comprising treating the acetyl cellulose with diphenyl black base in presence of acetic acid and at least one soluble 55 chloride salt and developing the dye on the acetyl cellulose.

7. Process for dyeing acetyl cellulose in black shades, comprising treating the acetyl cellulose with diphenyl black base in presence of acetic acid and protective colloid, and developing the dye on the acetyl cellulose.

8. Process for dyeing acetyl cellulose in black shades, comprising treating the acetyl cellulose with diphenyl black base in presence of acetic acid, at least one soluble chloride salt, and protective colloid, and developing the dye on the acetyl cellulose.

In testimony whereof I have hereunto 70 subscribed my name.

Dr. RENÉ CLAVEL.